

May 21, 1963

H. T. MINDEN ET AL

3,090,107

METHOD OF MAKING A PERMANENT MAGNET

Filed July 24, 1958



INVENTORS  
LEONARD BERENBAUM  
HENRY T. MINDEN  
BY *Leander J. J.*  
ATTORNEY

# United States Patent Office

3,090,107  
Patented May 21, 1963

1

3,090,107

METHOD OF MAKING A PERMANENT MAGNET  
Henry T. Minden, Roslyn Heights, and Leonard Berenbaum, Flushing, N.Y., assignors, by mesne assignments, to Sylvania Electric Products Inc., Wilmington, Del., a corporation of Delaware

Filed July 24, 1958, Ser. No. 750,725  
2 Claims. (Cl. 29—155.6)

This invention relates to improved permanent magnets. There are various applications which require the use of a permanent magnet having a very high coercive force. (The coercive force of a magnet is a measure of its ability to retain its magnetic strength under the influence of an opposing magnetic field.) For example, in certain traveling wave tube applications, a plurality of magnets having a general toroidal or washer shape are stacked in such manner that the resultant magnetic field is axial and adjacent faces of adjacent magnets have opposite magnetic poles. In order to produce the desired field strength, the magnets so shaped and so arranged must possess a high coercive force.

Conventional materials from which permanent magnets are made, such as Alnico V, lack the high degree of coercive force desired in the application described. Permanent magnets made of bismanol, however, do have the required high degree of coercive force, but corrode rapidly and suffer a permanent reduction in magnetic strength when exposed to a humid atmosphere not uncommonly encountered. Eventually the corrosion progresses to a point where cracking and pulverization of the magnet occurs, rendering it useless as a magnet.

Accordingly it is an object of our invention to produce an improved permanent magnet having a very high degree of coercive force so that it will retain its magnetic strength under the influence of demagnetizing fields.

Another object of this invention is to provide a method for making magnets having a higher coercive force than conventional magnetic materials and which will not be subject to corrosion, deterioration or cracking.

Still another object is to produce apparatus for making improved permanent magnets of the type herein described.

In accordance with the principles of our invention, a mixture of manganese bismuthide particles and a binder is placed in a non-magnetic container. This container is then placed in an apparatus where the binder is first subjected to a sufficient amount of heat to melt the binder material. While the binder is in a liquid state, pressure is applied to the mixture and simultaneously a magnetic field is applied to magnetically orient the particles of manganese bismuthide therein in the direction of the magnetic lines of force. The mixture is then cooled to solidify the binder while maintaining the pressure and the magnetic field. The container housing the magnet thus produced is then hermetically sealed to protect the magnetic substance from the atmosphere. A magnet is thus produced which has a very high coercive force and magnetic strength and which is not deleteriously affected by atmospheric conditions.

Our invention will now be described in detail with reference to the accompanying drawing which shows partly in cross section one embodiment of an apparatus employed to carry out the method of making the improved magnets.

Referring now to the drawing, there is shown a brass or other non-magnetic metallic container 10 toroidal in shape, which is lined with thin aluminum foil 11. A mixture 12 of manganese bismuthide and bismuth (bismanol) is then placed in the container and a flat cover 14 is placed over the container. The loaded container is

2

next placed on the top annular surface 15 of a lower die member 16 which has a central portion 18 extending into the center region of the toroidal container 10. This portion supports the inner sides of the container 10, when the mixture within the container is subjected to pressure as will later appear.

An upper die member 20 is next placed over the container cover 14 in alignment with the lower die member 16. The upper die member is provided with outer and inner annular grooves 24 and 26 respectively for receiving any molten overflow squeezed from the container 10 when heat and pressure are applied thereto in accordance with the method to be described. By providing annular grooves to collect the overflow, it is easier to break the container free from the upper die member when the process is complete. The central bore of the upper die member terminates at one end in a conical shape 28 to facilitate more even distribution of lines of magnetic flux through the upper die member 20. Lower and upper collar members 30 and 32 are disposed about the lower and upper die members 16 and 20 respectively, and support the external surface of container 10 when pressure is applied thereto.

Surrounding the upper and lower die members in the region of the container 10 is an electric heater 34 having wires 35 for heating the mixture in the container 10. A thermocouple 36 is located in the lower die member 16, which, in conjunction with an automatic controller (not shown) maintains the mixture at the proper temperature. Cooling coils 38 which carry circulating cold water are provided about the lower portion of the lower die member for cooling the mixture at the proper time. The cooling coils 38 are located some distance below the level of the container 10, so that the mixture can be cooled from the bottom of the container 10 rather than from its sides. Such directional cooling and the use of the aluminum foil 11 to eliminate sticking of the mixture to the inner wall of the container, prevent cracking of the magnet during the cooling process.

The upper and lower die member assembly just described is supported on the top face 39 of a lower pole piece 40, which is part of a large electromagnet comprising a lower pole piece 40, an upper pole piece 42, a yoke portion 44, and current carrying coils 46 disposed about both the upper and lower pole pieces. The upper yoke member 42 is slidably held by the yoke 44 to allow vertical movement thereof so that the face of the upper pole piece 42 can be brought into direct contact with the top 45 of the upper die member 20. Provision is also made to apply pressure vertically from a press, not shown, through a bar 48, the upper pole piece 42, upper die member 20 and the container cover 14, to compress the contents 12 in the container 10 thereby densifying the same.

The process is conducted in the following manner. The bismanol powder 12, which is composed of particles of manganese bismuthide and bismuth is loaded into the non-magnetic toroidal container 10. This is done under the protection of nitrogen to prevent reaction with the atmosphere. The cover 14 is then placed on the container 10. The loaded container is placed on the top surface 15 of the lower die member 16 which has disposed about it the lower collar 30, heater 34 and cooling coils 38. The upper die member 20 is then placed over the container cover 14, the upper collar 32 is placed in position and the upper pole piece 42 is lowered into contact with the top of the upper die member 20.

The heater 34 is then turned on and the temperature is automatically regulated by a controller in cooperation with the thermocouple 36. The mixture is heated to 300° C., a temperature above which bismuth melts

(271° C.) but below the Curie temperature of manganese bismuthide (360° C.), which is the temperature above which the latter material will lose its permanent magnetism.

While maintaining a temperature of 300° C., the manganese bismuthide particles become dispersed in the liquid bismuth medium and are magnetically oriented and then permanently retained in this position by freezing the liquid bismuth, as will now appear.

When the melting point of bismuth is reached, the magnetizing coils 46 are energized to create a strong magnetic field to thus magnetically orient the manganese bismuthide particles with respect to the direction of the applied magnetic field so that upon removal of the field, a strong permanent magnet will have been produced in the direction of the axis of the toroid. While the magnetic field is applied, the mixture is held at a temperature of approximately 300° C. In order to insure the proper orientation of all the manganese bismuthide particles, the magnetic field should be maintained for a sufficient time while the bismuth is molten. This time varies from several minutes for very thin magnets to several hours for very thick ones.

While the bismuth is molten, a pressure is applied through the bar 48 to increase the density of the contents of the container 10. The magnitude of the pressure is a variable depending upon the thickness of the magnet. After sufficient heating time has elapsed, the heater 34 is turned off and the container is cooled by passing cold water through the cooling coils 38. Cool air may also be blown over the apparatus to speed up the cooling process. To achieve maximum magnetic strength, it is important to maintain the magnetic field while the molten bismuth is above its melting point to insure that the manganese bismuthide particles are frozen in their properly oriented positions.

After the magnet is cooled, it is removed from the apparatus and sealed to protect the manganese bismuthide from the deleterious effects of the atmosphere. The sealing may be carried out by low temperature soldering or any other suitable method so long as the method does not result in melting of the bismuth or in otherwise decreasing the strength of the magnet.

By this method a permanent magnet is produced, which 45 has a high magnetic strength and also a much higher coercive force than conventional magnets. While our process has been described using bismuth as a binder to maintain the manganese bismuthide particles magnetically oriented in their proper positions, it should be 50 understood than other substances can also be used. For example, other non-magnetic metals having a melting point somewhat below 360° C., the Curie temperature of manganese bismuthide, would be suitable if they do not

react with the latter. Plastics and other compositions can also be used.

A modification of our process can be carried out by forming the magnet in the desired shape without the use of a container and subsequently sealing the magnet off from the deleterious effects of the atmosphere by the use of a protective coating.

What is claimed is:

- 10 1. The method of making a permanent magnet comprising, charging a toroidal container of non-magnetic material lined with aluminum foil and having a toroidal cover with a powder containing particles of manganese bismuthide and bismuth, heating said powder to a temperature sufficient to form a dispersion of manganese bismuthide particles in molten bismuth but below the Curie temperature of said manganese bismuthide, applying a magnetic field to said dispersion to magnetically orient said particles of manganese bismuthide with respect to said applied magnetic field, applying pressure between said toroidal cover and the bottom of said container to densify said solution, and directionally cooling said solution to solidify said bismuth while maintaining said manganese bismuthide particles so oriented, and hermetically sealing the cover on said container of non-magnetic material lined with aluminum foil, to protect the magnet so produced from the atmosphere.
- 15 2. The method of making a permanent magnet comprising dispersing particles of a ferromagnetic material in a liquid binder held in a non-magnetic container having a cover, said binder being held at a temperature sufficient to maintain said binder in a liquid state but below the Curie temperature of said ferromagnetic material, subjecting said ferromagnetic material to the influence of a magnetic field to magnetically orient said ferromagnetic particles with respect to the direction of said applied magnetic field, densifying said dispersion, directionally cooling and freezing said binder while maintaining said ferromagnetic particles so oriented to permanently fix said particles in said oriented direction, and sealing the cover on said container of non-magnetic material to protect its contents from the atmosphere.

References Cited in the file of this patent

UNITED STATES PATENTS

|           |                |       |               |
|-----------|----------------|-------|---------------|
| 2,576,679 | Guilland       | ----- | Nov. 27, 1951 |
| 2,589,766 | Bradley        | ----- | Mar. 18, 1952 |
| 2,698,917 | Van Urk et al. | ----- | Jan. 4, 1955  |
| 2,751,525 | Hekelaar       | ----- | June 19, 1956 |
| 2,825,670 | Adams et al.   | ----- | Mar. 4, 1958  |
| 2,849,312 | Peterman       | ----- | Aug. 26, 1958 |
| 2,862,287 | Koch et al.    | ----- | Dec. 2, 1958  |
| 2,865,085 | Cornish        | ----- | Dec. 23, 1958 |
| 2,892,248 | Weber et al.   | ----- | June 30, 1959 |